

May 1, 1945.

A. BEERBOWER ET AL

2,374,913

PREPARATION OF LUBRICATING GREASES AND APPARATUS THEREFOR

Filed Aug. 15, 1941



Alan Beerbower Inventor  
John C. Zimmer  
By *P. H. Young Attorney*

## UNITED STATES PATENT OFFICE

2,374,913

PREPARATION OF LUBRICATING GREASES  
AND APPARATUS THEREFOR

Alan Beerbower, Kenilworth, and John C. Zimmer, Union, N. J., assignors to Standard Oil Development Company, a corporation of Delaware

Application August 15, 1941, Serial No. 406,988

10 Claims. (Cl. 252—39)

This invention relates to novel methods for producing lubricating greases and soap stocks or concentrates for the manufacture of greases and to novel apparatus therefor; and more particularly it relates to a novel and improved process and apparatus for continuously making a lubricating grease soap concentrate which can then be compounded with the required proportion of mineral oil, with the result that a completely continuous process for making lubricating greases from start to finish is made possible by an improved process which attains high quality products at relatively much lower cost than processes used heretofore.

The invention has been found particularly applicable to the manufacture of calcium soap greases and will first be described as such. For producing calcium soap concentrate which is to be used for making lime base greases, a saponifiable material, such as the usual animal fat, is mixed with the saponifying agent, preferably hydrated lime, with or without a small amount of water and/or a small amount of a mineral oil, and this mixture, preferably in the form of a semi-fluid paste, is passed continuously in a relatively small stream through a heating zone where the temperature of the mixture is raised at least to saponification temperature, then the mixture is maintained at a temperature at least as high as the saponification temperature until saponification is substantially complete and there is thus continuously produced a calcium soap concentrate suitable for grease making which may then either be passed to a storage zone or preferably, immediately compounded either continuously or by batch operation with the required proportion of mineral oil to produce a lime-soap lubricating grease of uniform and high quality.

The invention will be better understood by referring to the accompanying schematic drawing showing a complete grease-making apparatus consisting essentially of a mixing chamber 1, a heater 2, a reaction-completing zone 3, together with alternate batch or continuous equipment 4 or 5, respectively, for blending the soap concentrate discharging from the reaction-completing zone 3 with the required amount of mineral oil of desired grade (A, B, C, D, or E, etc.) from suitable supply sources not shown. In carrying out the invention, the mixing zone 1 is preferably charged continuously by feeding the fat or other suitable saponifiable material through line 6, the hydrated lime or other saponifying agent through line 7 (either dry or

5 admixed with a small amount of water as a slurry, although the water may be fed in separately, if desired) and the mineral oil through line 8, although, if desired, the soap concentrate may be prepared without the use of any mineral oil. The mixing zone may be of any suitable type, such as the vertical cylindrical mixing chamber 1, equipped with an agitator as illustrated in the drawing, or it may be in various other forms not shown, such as a screw conveyor or even a simple or baffled pipe in which the various materials become mixed by turbulent flow through the pipe.

10 Also if desired, this mixing may be accomplished in a semi-continuous manner by using two or more batch mixing tanks operated alternately or in series so that while one is being continuously fed into the heater 2, one or more others may be used for mixing new batches; in this manner a continuous supply of cold saponification mixture may be made available for continuous feeding into the heater 2. The mixture to be saponified, e. g., hydrated lime and fat, preferably also containing a small amount of water and of mineral oil, is then forced through line 9 by pump 10 into heater 2, illustrated in the drawing as consisting of a steam-heated coil of pipe. Obviously, the number of tubes or length of pipe used in such a coil heater may be varied according to the speed of flow desired and the degree of heat available, as a single straight tube may be sufficient if a high enough steam pressure is used and a small enough tube diameter or slow enough flow through the tube is used. As an example of designing this feature of the invention, it may be mentioned that an overall heat transfer coefficient of 35 B. t. u. per hour per square foot per degree Fahrenheit may be obtained. This means, specifically, that a steam gauge pressure of about 100 pounds per square inch would be sufficient to heat a saponification mixture from a room temperature of about 95° F. up to about 320° F. when pumped through a 1½-inch inside diameter tube having a total heated length of 105 feet at the rate of 15 pounds per minute.

15 The heating of the heater 2 may be accomplished by various means other than steam, for instance, by fused salt, diphenyl oxides, mixtures of diphenyl oxide and diphenyl, etc. or by direct firing of suitable tubes or pipe coils. A screw conveyor can be used for forcing the saponification mixture through heating tubes, if desired, the latter being heated either by steam or direct fire.

If desired, the temperature maintained in the heater 2, may be so controlled in relation to the size and length of tubing therein as to effect a complete saponification before issuing from the heater per se, if desired, or alternatively, as shown in the drawing, the saponification mixture may be merely rapidly heated in heater 2 as, for instance, in a period of less than 10 minutes, to a temperature at least as high as the saponification temperature, namely, to a minimum of 250° F. and preferably to 300 or 400° F. or even higher, in some cases even as high as 550° F., and then immediately passed through line 11 to a summation zone or a reaction-completing zone 3 which may or may not be heated, but if not heated, is insulated or so designed to maintain a sufficient amount of the heat in the saponification mixture to effect the completion of the saponification reaction. In the drawing, this reaction-completing zone 3 is illustrated as being a tank of substantial volume into which the heated saponification mixture is charged at the top and discharged continuously at the bottom. Obviously other shapes and types of equipment may be used as a reaction-completing zone. For instance, this result may be accomplished by using a long tube or coil of pipe, either heated slightly or insulated to prevent cooling, and designed of sufficient length that when the soap stock is discharged therefrom, the saponification reaction will have been substantially completed, i. e., at least to the extent of 95%, and preferably to at least 98%. In the above hypothetical example, the reaction-completing chamber should be of about 60 gallons working capacity. The reaction-completing zone may be provided, if desired, or necessary, with suitable baffles to prevent channelling of the soap stock while passing therethrough. The reaction-completing zone 3 is preferably provided with a safety valve 13 to provide for release of vapors in case dangerously or undesirably high pressures are developed in this soap-stock manufacturing equipment, though no vapors should be removed in ordinary operation with lime soap greases. Normally, in the production of a calcium soap stock for lubricating grease manufacture, it is desirable to operate the whole system under a superatmospheric pressure of, for instance, 15 to 250 pounds per square inch, in order to facilitate hydrolysis of glycerides and to retain in the soap concentrate a sufficient proportion of water to assist in forming the proper grease structure when the soap concentrate is finally compounded with the main body of mineral oil.

When the finished soap concentrate issues continuously from the reaction-completing zone 3, it may either be passed directly to storage through line 14, or passed through line 15 into one of the two alternative grease-blending units 4 and 5, 4 being shown in the drawing as a batch-operated mixing tank equipped with an agitator and provided with a soap-concentrate inlet and a mineral oil inlet at the top and a discharge outlet 16 at the bottom. The blending unit 5 is shown in the drawing as composed of two gear pumps or other suitable metering devices 17, one for the soap stock and the other for the mineral oil fed from suitable sources A, B, C, D, or E, and a high-speed mixer 18, as claimed in co-pending application Serial Number 342,081, filed June 24, 1940, now Patent Number 2,318,668, granted May 11, 1943, preferably of the Lancaster mixer type for final discharge through outlet 19. Outlets 16 and 19 should be provided with pres-

sure-controlled valves so as to maintain the entire system including the heater, reaction-completing zone and blending unit under the desired operating pressure. Obviously the mineral oil from source A, B, C, D, or E may be preheated, if desired, in order to obtain the proper temperature in the blended grease for facilitating homogeneous dispersion of the soap within the oil and production of the proper grease structure.

- 10 As indicated in the drawing, the mixer 1 may be provided with a line 20 for temporarily recycling the cold saponification mixture through the mixer 1, at least long enough to insure that a substantially homogeneous mixture will be fed into 15 the heater 2. The equipment is provided with suitable valves, such as indicated in the drawing, for controlling the flow or stoppage of the saponification mixture, as required for normal operation as described, with proper means for dis- 20 charging and cleaning the various parts of the apparatus when necessary.

The saponifiable material to be used may be any of the fats, fatty oils, fatty acids, etc., commonly used for making lubricating grease. Specific examples of such materials include beef 25 stearin, mutton tallow, hog fat, lard oil, cotton-seed oil, soya bean oil, oleic, stearic or tallow fatty acids, or degreas. Of these various types of 30 saponifiable material hog fat, lard oil and the various fatty acids are preferred, especially for making lime soap greases.

As the saponifying agent, lime is preferred and this may be used either in the form of calcium hydroxide or calcium oxide, although the former 35 is preferred. Other alkaline earth metal bases of periodic Group II-A may be used, such as gelatinous magnesium hydroxide and corresponding strontium and barium hydroxides or oxides. Although the invention is particularly applicable to 40 the preparation of alkaline earth metal soap greases, other saponifying agents may be used, such as caustic soda, caustic potash, caustic lithium, gelatinous aluminum hydroxide, or mixtures of two saponifying agents such as lime and 45 soda, lime and potash, soda and barium, lime and barium, etc., in which the metal outside Group II-A is less than 10% of the base.

The saponification of fats to make a grease 50 concentrate by long cooking continuously has already been suggested as in U. S. Patent No. 2,084,974. This invention, however, is different in that complete and efficient mixing is effected before heating and therefore the time of reaction 55 is much shorter, namely from  $\frac{1}{4}$  to  $1\frac{1}{2}$  hours and also differs in other important features.

As indicated earlier, it is desirable with certain 60 types of greases, particularly the lime greases, to have a small amount of water present in order to obtain the best grease structure and the optimum yield, expressed in volume of grease produced for any particular soap content. For lime soap greases, it is preferable to have a water content between the approximate limits of 0.5 and 5.0% in the finished grease composition, or approximately 0.10% of water for each per cent of lime soap present. If the saponifiable material used is a glyceride or a mixture of glycerides, 65 some glycerine is formed as a by-product of the saponification reaction, and whatever water is desired in the finished grease must be added. On the other hand, if fatty acids are used as the saponifiable material, then some water is formed 70 as by-product during the saponification, and in

such a case little, if any, additional water need be added.

As referred to earlier, it is possible to make various soap concentrates without having any mineral oil present, but it is preferred to prepare the soap stock in the presence of a small amount of mineral oil, usually less than 30% of the weight of saponifiable material, and preferably about 10-20% of the weight of saponifiable material. The mineral oil for this purpose may be of any particular type, as to whether it is paraffinic, naphthenic, or mixed base oil, or of the particular boiling range and viscosity range intended to be used in the finished grease composition, or, since only a relatively small amount of the oil is used in making the concentrated soap stock, a medium type of mineral lubricating oil may be used for this purpose, e. g., one having a Saybolt viscosity between the approximate limits of 40 seconds and 60 seconds at 210° F., this soap concentrate then being blended with a much larger proportion of a mineral oil of the desired characteristics for making the finished lubricating grease. The oil used in the soap concentrate should be of as light a color as any oil to be used in blending.

For the sake of illustration, the following example is given.

The materials listed herebelow were mixed at ordinary room temperature (the quantities being expressed in per cent by weight) and formed a semi-fluid paste:

| Material                                       | Per cent |
|------------------------------------------------|----------|
| Commercial hog fat                             | 75       |
| Hydrated lime (chemical grade)                 | 10.5     |
| Water                                          | 7.5      |
| Mineral oil of 40 S. S. U. paraffin at 210° F. | 7.0      |
|                                                | 100.0    |

The above mixture must be used within 24 hours, because if it stands longer, it sets practically solid. These materials were mixed in a mixer such as illustrated at 1 in the accompanying drawing, and the resultant slurry was pumped through the heater 2, whereby it was raised to a temperature of about 320° F. in about 5 minutes, and then it was admitted at the top of the reaction-completing chamber 3, its course through the latter taking at least an hour, after which it was withdrawn from the bottom of the reaction-completing chamber at the same rate at which it was charged in at the top. The heater coil was 20 feet of  $\frac{1}{4}$  inch inside diameter tubing immersed in an oil bath at 320° F. The feed rate was 60 grams per minute. The reaction-completing zone was 4 inches inside diameter and 12 inches high, mounted vertically in a tank of hot oil at 320° F. It was not fitted with baffles nor any stirring mechanism. One analysis during this continuous grease soap concentrate manufacture indicated that the saponification was 98.7% complete, and this compares very favorably with the 95-98% ordinarily obtained in batch operations.

The soap concentrate produced in this test was, when cooled, a hard, brittle material of approximately 10 penetration by the A. S. T. M. grease penetration test. It had a melting point of 210° F. If melted under pressure it becomes a viscous fluid, thinning as the temperature is raised. At 300° F. it flows quite freely.

Several different greases were blended from the above concentrate, including two containing

oil having a viscosity of 40 seconds Saybolt (Univ.) at 210° F. of 225 and 300 worked penetration, and one with oil having a viscosity of 70 seconds Saybolt at 210° F., of 300 worked penetration.

It is not intended that this invention be limited to the specific examples recited, nor to the particular types of equipment shown in the accompanying drawing which are given merely for illustration, but only by the appended claims in which it is intended to claim all novelty inherent in the invention.

We claim:

1. The process of preparing a lubricating grease soap concentrate which comprises mixing in a mixing zone of relatively large capacity a saponifiable material, a saponifying agent in substantial amounts to completely saponify the saponifiable material and a small amount of mineral oil, at a temperature lower than saponification reaction temperature but sufficiently high to maintain the mixture in a semifluid or fluid state and to permit thorough mechanical mixing, continuously heating the resulting mixture in a small stream in a heating zone of relatively small capacity compared to that of the mixing zone to a temperature at least as high as saponification reaction temperature, maintaining said mixture at a temperature at least as high as reaction temperature until the saponification reaction is substantially complete, and continuously withdrawing the finished lubricating grease soap stock.

2. Process according to claim 1 in which an alkaline earth saponifying agent is used and the saponification mixture is heated in a confined stream for a period of less than 10 minutes.

3. Process according to claim 1 in which animal fat and hydrated lime are used, the saponification mixture is heated to about 300° F. to 450° F. in a pipe coil heater in less than about 10 minutes, and the saponification mixture is then kept at reacting temperature for at least one quarter hour.

4. The process of preparing a lubricating grease soap stock which comprises mixing at room temperature the following amounts of materials, expressed in percent by weight:

| Material      | Per cent |
|---------------|----------|
| Animal fat    | 50-80    |
| Hydrated lime | 7-12     |
| Water         | 5-8      |
| Mineral oil   | 0-35     |

continuously heating said mixture to about 300-400° F. in a pipe coil for less than about 10 minutes, maintaining the mixture at a temperature at least as high as 250° F. for at least one quarter hour while continuously passing it through a reaction-completing zone, said mixture being kept under a sufficient pressure to prevent undue evaporation of water while hot, and continuously withdrawing from the reaction-completing zone a finished lubricating grease soap stock.

5. The process of preparing a lubricating grease soap stock which comprises continuously mixing in a mixing zone of relatively large capacity a saponifiable material, a saponifying agent and a small amount of mineral oil, at a temperature lower than saponification reaction temperature but sufficiently high to maintain the mixture in a semifluid or fluid state and to permit thorough mechanical mixing, continuously withdrawing a portion of said mixture from said mixing zone,

continuously heating said mixture in a small stream in a heating zone of relatively small capacity to a temperature at least as high as saponification reaction temperature, maintaining said mixture at a temperature at least as high as reaction temperature until the saponification reaction is substantially complete, and continuously withdrawing the finished lubricating grease soap stock.

6. The process of preparing a lubricating grease which comprises continuously mixing a saponifiable material, a saponifying agent and a small amount of mineral oil at a temperature lower than saponification reaction temperature but sufficiently high to maintain the mixture in a semifluid or fluid state and to permit thorough mechanical mixing, continuously heating said mixture in a small stream to a temperature at least as high as saponification reaction temperature, maintaining said mixture at a temperature at least as high as reaction temperature until the saponification reaction is substantially complete, continuously withdrawing a finished lubricating grease soap concentrate, and compounding the resulting soap concentrate with a major proportion of mineral oil to make a finished lubricating grease.

7. The process of preparing a lubricating grease which comprises continuously mixing a saponifiable material, a saponifying agent and a small amount of mineral oil at a temperature lower than saponification reaction temperature but sufficiently high to maintain the mixture in a semifluid or fluid state and to permit thorough mechanical mixing, continuously heating said mixture in a small stream to a temperature at least as high as saponification reaction temperature, maintaining said mixture at a temperature at least as high as reaction temperature until the saponification reaction is substantially complete, continuously withdrawing a finished lubricating grease soap concentrate, and continuously compounding the resulting soap concentrate with a major proportion of mineral oil to make a finished lubricating grease.

8. A continuous process for making a calcium soap lubricating grease which comprises continuously mixing at about room temperature the following proportions of materials by weight:

| Material           | Per cent |
|--------------------|----------|
| Animal fat.....    | 50-86    |
| Hydrated lime..... | 7-12     |
| Water.....         | 5-8      |
| Mineral oil.....   | 0-35     |

continuously heating the resulting mixture to about 300-400° F. in a steam-heated pipe coil in a short time of less than about 10 minutes, continuously passing the heated mixture through a

5 reaction-completing zone where the temperature of said mixture is kept at least as high as saponification temperature until the saponification is substantially complete, and continuously blending the resultant calcium soap stock with additional mineral lubricating oil, said materials being kept under a sufficient superatmospheric pressure while hot to prevent undue vaporization of water.

9. The process of preparing a mineral lubricat-

15 ing oil grease which comprises mixing a saponifiable material and a saponification agent at a temperature lower than saponification reaction temperature but sufficiently high to maintain the mixture in a semifluid or fluid state and to permit

20 thorough mechanical mixing, continuously heating said mixture in a small stream to a temperature at least as high as saponification reaction temperature, maintaining said mixture at a tem-

25 perature at least as high as reaction temperature until the saponification is substantially complete, continuously withdrawing a soap stock, and compounding said resulting soap stock with a mineral lubricating oil to make a lubricating grease.

30 10. A continuous process for making a lubri-

cating grease soap stock which consists essen-

35 tially in continuously feeding into a mixing zone of relatively large capacity a saponifiable ma-

terial, a saponifying agent in sufficient amount to substantially completely saponify said saponifi-

40 able material, and a small amount of mineral oil, continuously mixing said materials in said mixing zone, with a mechanically operated agi-

45 tator at a temperature lower than saponification reaction temperature but sufficiently high to maintain the mixture in a semifluid or fluid state and to permit thorough mechanical mixing, continuously withdrawing a portion of said mixture from said mixing zone and continuously heating

45 it in a once-through operation in a small stream in a heating zone of relatively small capacity to a temperature at least as high as saponification reaction temperature and maintaining said mixture at a temperature at least as high as saponi-

50 fication temperature until saponification is sub-

stantially complete.

ALAN BEERBOWER.  
JOHN C. ZIMMER.